

# UNITED STATES PATENT OFFICE.

OLIVER P. M. GOSS, OF SEATTLE, WASHINGTON.

## ART OF IMPREGNATING TIMBER AND OTHER MATERIAL WITH A PRESERVATIVE.

1,219,550.

Specification of Letters Patent. Patented Mar. 13, 1917.

No Drawing.

Application filed October 11, 1915. Serial No. 55,577.

*To all whom it may concern:*

Be it known that I, OLIVER P. M. Goss, a citizen of the United States, and a resident of Seattle, county of King, State of Washington, have invented a certain new and useful Improvement in the Art of Impregnating Timber and other Material With a Preservative, of which the following is a specification.

10 My present invention is particularly concerned with the treatment of timber, such as railroad ties, paving blocks, woodstave pipes, special kinds of lumber, and the like, and it has for its special object the producing of ties which conform with the demands of the market at the present time, that is, ties which have been efficiently, but not wastefully, impregnated with the preserving material, and furthermore are thoroughly surface dry.

In order to fully attain my object I preferably pursue the following method: I place the timber to be treated in a retort made with a door adapted to be hermetically sealed. Then I introduce a preservative such as coal tar, creosote, or other bituminous liquids into the retort, after which I heat the preservative to a temperature of approximately 230 degrees Fahrenheit under normal pressure; then I draw a vacuum of from 15 to 28 inches in the retort; then, without disturbing such vacuum in the retort, I maintain the heat of the latter at a temperature above that of boiling water under such vacuum, for not less than one-half hour. Then I break the vacuum in the retort, and then apply pressure on the fluid in the retort sufficient to force into the pores of each cubic foot of the material being treated approximately from 5 to 20 pounds of the fluid.

In order to render the surface of the treated material dry, the following additional steps must be taken. Reheat the fluid in the retort from 1 to 6 hours additional to the temperature of from 200 to 240 degrees Fahrenheit, then empty the retort of the preserving fluid; and, finally, while the material is still in the retort, and hot, draw the vacuum in the latter of from 15 to 28 inches. By this process the surplus preservative will be drawn out of the pores of the material and the latter thus renders the surface dry. The reheating of the preservative will cause the gases in the pores to expand and thus facilitate the rejection of

the surplus preservative when the final vacuum is drawn. When the material is finally taken from the retort and cooled, the contraction of the gases in the pores will tend to draw the remaining preservative well into the pores and thus leave the surface of the material dry.

The above described process will not be sufficient to insure the thorough penetration of the preservative into the pores of some material. In this case the following procedure should be substituted for the steps outlined in the foregoing paragraph. Reheat the fluid in the retort for from 1 to 6 hours, continuously, to a temperature of from 200 to 240 degrees Fahrenheit under normal pressure; then draw a vacuum of from 15 to 28 inches on the preserving fluid in the retort, then, while still under such vacuum, continue the heat above the boiling point of water under the vacuum for not less than one-half hour, then break said vacuum and empty the retort of the preserving fluid; and, finally, while the material is still in the retort, and hot, draw a vacuum in the latter of from 15 to 28 inches approximately.

In describing my process I have necessarily to avail myself of a wide range in the degree of heat, in the vacuum produced, and in the length of time during which a specific treatment is carried on, for it is impossible to be more specific in these details, since different materials have different natures and require corresponding variation of their treatment. These specific details must, in the first instance, be determined for the different materials by a preliminary trial.

In short, the variations of my process are for the purpose of limiting the work done on the material to that required, in order to attain the best results, in which the following is essential: First, the thorough expulsion of moisture from the timber, second, the forcing of sufficient preservative well into the pores of the material, and lastly, the ejection of surplus preservative so that the surface of the treated material will be dry, which conditions are generally demanded by the market.

I claim:

In the preserving treatment of porous material, the method which consists in first heating the material in a bituminous preservative, in a closed container, to approximately 230 degrees Fahrenheit under normal

pressure, then drawing a vacuum of approximately 15 to 28 inches in the container and maintaining the heat of the latter at a temperature above that of boiling water under said vacuum for not less than half an hour, then breaking such vacuum, and applying pressure sufficient to force approximately from five to twenty pounds of the preservative fluid into the pores of each cubic foot of material.

10 2. In the preserving treatment of porous material, the method which consists in first heating the material in a bituminous preservative, in a closed container, to approximately 230 degrees Fahrenheit under normal pressure, then drawing a vacuum of approximately 15 to 28 inches on the preserving fluid and continuing to heat the latter to a temperature above that of boiling water under said vacuum, for not less than half an hour, then breaking such vacuum, and applying pressure sufficient to force approximately from 5 to 20 pounds of the preservative fluid into the pores of each cubic foot of material, then reheating the fluid in the container for from one to six hours continuously to a temperature of from 200 to 240 degrees Fahrenheit under normal pressure, then emptying the container of the preserving fluid, and then, while the material is

15 still hot, drawing a vacuum in the container of from 15 to 28 inches approximately.

3. In the preserving treatment of porous material, the method which consists in first heating the material in a bituminous preservative, in a closed container, to approximately 230 degrees Fahrenheit under normal pressure, then drawing a vacuum of approximately 15 to 28 inches on the preserving fluid and continuing to heat the latter to a temperature above that of boiling water under said vacuum, for not less than half an hour, then breaking such vacuum, and applying pressure sufficiently to force approximately from 5 to 20 pounds of the preservative fluid into the pores of each cubic foot of material, then reheating the fluid in the container for from one to six hours continuously to a temperature of from 200 to 240 degrees Fahrenheit under normal pressure, then drawing a vacuum of 15 to 28 inches on the preserving fluid and boiling in the fluid under this vacuum for not less than one hour, then breaking such vacuum, and emptying the container of the preserving fluid, and then, while the material is still hot, drawing a vacuum in the container of from 15 to 28 inches approximately.

O. P. M. GOSS.